

# United States Patent Office

3,501,304  
Patented Mar. 17, 1970

11

**3,501,304**  
**PHOTOGRAPHIC GELATINOUS LIQUID**  
**COMPOSITIONS**

Kenichi Koda, Tokyo, Sadao Sugita, Hanno-shi, and  
Shoji Kikuchi and Katsumi Nishimura, Tokyo, Japan,  
assignors to Konishiroku Photo Industry Co., Ltd.,  
Tokyo, Japan, a corporation of Japan.

Tokyo, Japan, a corporation of Japan  
No Drawing. Filed Mar. 7, 1967, Ser. No. 621,131  
Claims priority, application Japan, Mar. 17, 1966.

Claims priority, application Japan,  
41/16,095  
Int. Cl. G03c 1/02

## 2 Claims

## ABSTRACT OF THE DISCLOSURE

Photographic gelatinous liquid compositions containing as an anti-foaming agent a compound of the general formula



wherein  $n$  is an integer of 3 or 4 and  $m$  is an integer of not less than 5.

This invention relates to a photographic gelatinous liquid composition, characterized by that said composition contains a compound of the general formula



wherein  $n$  is an integer of 3 or 4 and  $m$  is an integer of not less than 5. More particularly, this invention is concerned with use of a new defoaming and anti-foaming agent in a photographic gelatinous emulsion or solution. It is accordingly an object of the invention to provide a substantially foam-free photographic gelatinous emulsion or solution which enables us to prepare a light-sensitive photographic material efficiently and economically.

In the preparation of light-sensitive silver halide photographic materials, handling of a gelatine-containing liquid composition (emulsion or solution) is a very common work. It is necessary to handle such composition, for example, in the step of preparing an aqueous gelatine solution, the step of adding a water-soluble halide and a 45 water-soluble silver salt (silver nitrate) to the aqueous gelatine solution and the step of coating the resulting emulsion onto a support. As is well known, the gelatinous emulsion or solution is very liable to cause foaming, which often raises serious problems in process operations. For instance, the emulsion components are not dissolved completely nor dispersed uniformly, due to the foams formed by said phenomenon. Further, in forming a silver halide by adding a halide and a silver salt to an aqueous gelatine solution, a heterogeneous reaction takes place in the 55 vicinity of the liquid surface due to the foams, with the result that coarse silver halide particles, so-called coarse grains, are formed, which will be a cause for undesirable fogging. In addition, when an emulsion involving foams is coated onto a support, the resulting layer unavoidably suffers from unevenness or comet, which are detrimental to the photographic product.

Furthermore, the foaming phenomenon is a great obstacle when the increased production of a light-sensitive photographic material is intended. For example, in case the rotation of a stirrer is sped up, the foaming becomes so vigorous that the content to be stirred is overflowed.

2

out of the vessel together with the foams. Further, the foams once formed do not disappear in a short period, and therefore it is difficult by visual inspection to confirm whether or not the emulsion components (e.g., gelatine, halide and silver nitrate) have been dissolved. Moreover, the apparatus employed is required to have a space corresponding to the anticipated amount of foams, and hence should uneconomically be made larger in scale.

In order to dismiss such a foaming phenomenon as mentioned above, various defoaming agents have been proposed. However, these defoaming agents are still unsatisfactory. For example,  $C_5-C_8$  alcohols are required to be used in large quantities because of their insufficient defoaming activity. Further, use of such alcohols in a photo-film plant is very hazardous because the operations in said plant are effected chiefly in closed room and these alcohols are vaporizable. Silicon oils are excellent in defoaming effect but, in the coating step, they bring about a so-called repelling phenomenon to lower the quality of the products.

20 We have found that a compound of the above-defined general formula is very effective as a defoaming and anti-foaming agent for use in a photographic gelatinous liquid composition. In the photographic art, undesired foaming  
25 is inherent to a gelatine-containing emulsion or solution which may be light-sensitive or not. Thus, the compound disclosed as a defoaming and anti-foaming agent in this invention is useful for any gelatine-containing liquid composition used in the photographic art, for example, including photographic light-sensitive gelatino silver halide emulsions, direct positive light-sensitive gelatino silver halide emulsions (which contain fogged silver halide crystals) and non-light-sensitive gelatine-containing emulsions or solutions to be used for coating of subbing layer, intermediate layer, anchoring layer and other auxiliary layer.  
30 In the following description, our reference sometimes will be made with reference to the foaming of a light-sensitive gelatino silver halide photographic emulsion. However, it should be understood that such description is informative  
35 only and the principle of the invention is applicable, with success, to any photographic liquid composition as far as it suffers from foaming due to the action of gelatine.  
40

The compounds of the aforesaid general formula are excellent not only in defoaming and anti-forming properties but also in surface active properties. Thus, they further serve as surface tension depressants for photographic emulsions or solutions, without any adverse effect on the photographic characteristics of the said photographic emulsions or solutions. If a compound of the above general formula is incorporated in an aqueous solution containing a foaming surface active agent with undesired foaming property, not only the foaming action of the surface active agent is decreased but also foams once formed are destroyed. Therefore, when used in combination with saponin or sodium isoamyldecylsulfosuccinate, both of which are excellent in spreadability but have frequently brought about various drawbacks due to their foamability, the compound of the above general formula inhibits the foaming without injuring the preferable characteristic of said substance, i.e. spreadability, and remove the foams once formed.

A compound of the above-indicated general formula can be prepared, in general, by condensing 2 mols of epichlorohydrin with one mol of polyalkylene glycol in the presence of an acidic catalyst (e.g. Lewis acid), epoxidizing the resulting polyoxyalkylene-bis-(3-chloro-2-oxy-propyl)-ether with an alkali and then hydrolyzing said

ether with an aqueous acid or alkali solution. Typical examples of the compounds are set forth below:

invention is found to be excellent in surface tension-depressing ability.

| No.      | Number of n | Number of m | Elementary analysis |        |       |        |           |        |       |        |            |        |                     |        |
|----------|-------------|-------------|---------------------|--------|-------|--------|-----------|--------|-------|--------|------------|--------|---------------------|--------|
|          |             |             | C percent           |        |       |        | H percent |        |       |        | OH percent |        | Average mol. weight |        |
|          |             |             | Found               | Calcd. | Found | Calcd. | Found     | Calcd. | Found | Calcd. | Found      | Calcd. | Found               | Calcd. |
| I-----   | 3           | 7           | 56.41               | 56.62  | 9.86  | 9.86   | 11.74     | 11.88  | 580   | 573    |            |        |                     |        |
| II-----  | 3           | 12          | 58.31               | 58.44  | 10.15 | 10.04  | 7.69      | 7.88   | 885   | 863    |            |        |                     |        |
| III----- | 3           | 17          | 58.93               | 58.83  | 10.05 | 10.91  | 5.60      | 5.85   | 1,210 | 1,164  |            |        |                     |        |
| IV-----  | 3           | 34          | 60.10               | 60.30  | 10.23 | 10.69  | 3.09      | 3.16   | 2,200 | 2,151  |            |        |                     |        |
| V-----   | 3           | 52          | 61.21               | 61.06  | 10.16 | 10.31  | 2.04      | 2.14   | 3,330 | 3,186  |            |        |                     |        |
| VI-----  | 4           | 7           | 60.98               | 60.86  | 10.36 | 10.52  | 9.98      | 10.14  | 680   | 671    |            |        |                     |        |
| VII----- | 4           | 14          | 63.22               | 63.34  | 10.65 | 10.80  | 5.54      | 5.79   | 1,230 | 1,176  |            |        |                     |        |

In accordance with the present invention, such compound as mentioned above is used, either as such or in the form of a solution in water or in a water-soluble organic solvent, such as a lower alcohol, at an optional stage or stages in the steps for the production of light-sensitive silver halide photographic materials. The amount of the compound added is most preferably about 0.01-10 g. per liter of the photographic emulsion or solution to which the compound is to be added, but the amount is more or less variable in some cases. The compound is preferably added prior to the step at which the formation of foams is anticipated, but it is not objectionable that the compound is directly sprayed over a portion in which foams have been formed. For example, in the case where an aqueous gelatine solution is to be prepared, the compound may have previously been incorporated in a given amount of water into which gelatine is to be dissolved, or may be added while gelatine is under stirring and dissolution.

When the compound is used for a light-sensitive gelatino silver halide photographic emulsion, it may preferably be added either before, during or after the ripening or may be added to a supernatant formed during the precipitation of light-sensitive silver halide crystals. According to this way, a light-sensitive gelatino silver halide photographic emulsion can be made free from undesired foaming, without any injury of its photographic characteristics at all, with the result that it is possible to produce a light-sensitive silver halide photographic material excellent in quality at an improved production efficiency.

In order to demonstrate the effectiveness of the compounds disclosed herein, our explanation will be given in connection with the following tests:

#### (A) SURFACE TENSION TEST

Compound (IV) which is shown in the above table and, as a control, a polyoxypropylene-polyoxyethylene glycol, in which the polyoxypropylene portion has an average molecular weight of 1000 and the polyoxyethylene portion consists of 20% by weight of the total molecular weight (Pluronics), were prepared, respectively, into 0.001%, 0.01% and 0.1% aqueous solutions. The solutions were measured in surface tension by using a Du Noüy's tension meter to obtain the results as shown below.

| Agent used         | Temperature (°C.) | Surface tension (dyne/cm.) |       |      |
|--------------------|-------------------|----------------------------|-------|------|
|                    |                   | 0.001%                     | 0.01% | 0.1% |
| Compound (IV)----- | 20                | 43.4                       | 37.7  | 33.8 |
| Control-----       | 25                | 53.6                       | 47.5  | 41.1 |

As shown in the above, the compound of the present

75

The foaming state of the emulsion was observed to recog-

#### (B) FOAMING TEST

The compound (VII) and as a control, the polyoxypropylene-polyoxyethylene glycol used in the above test A were tested in defoamability and antifoamability.

25 50 ml. of a 7% aqueous gelatine solution was charged in a 100 ml. cylinder. Into the solution, 4 ml. of a 1% aqueous solution of each of the above-mentioned compound (VII) and glycol was incorporated, and the mixed solution was shaken at 40° C. Foaming was measured in term of foam volume. The results are set forth below.

| Agent used          | Volume of foams (ml.) |              |
|---------------------|-----------------------|--------------|
|                     | After 1.5 min.        | After 5 min. |
| Not added-----      | 32                    | 27           |
| Compound (VII)----- | 1                     | 0.5          |
| Control-----        | 4                     | 3            |

As is clear from the above table, the compound of the present invention is markedly excellent in defoaming and anti-forming properties.

40 The following examples describe certain ways in which the principle of the invention has been applied, but are not to be construed as limiting its scope.

#### Example 1

45 Into a cylindrical vessel of 1 m. in diameter and 2 m. in height, 10 kg. of photographic gelatine and 1000 l. of water (deionized) were charged and the gelatine was swelled. To the vessel, 200 g. of the compound (II) was added, and the mixture was stirred at a speed of 300 r.p.m. for 30 minutes while maintaining the temperature at 50° C. The height of foams formed on the emulsion was measured to obtain the following result, which is shown in comparison with the case where the compound (II) was not used.

55 Height of foams, cm.  
Incorporated with compound (II) ----- 0.2  
Not incorporated with compound (II) ----- 5

60 The run in which the compound (II) was used could be carried out little foams which disappeared within 1 minute, whereas the control run suffered from marked foams which did not disappear even after 5 minutes. In the latter case, it was difficult to visually confirm the dissolution of gelatine. In the former case, no increase in foaming was observed even when the stirring speed was elevated to 500 r.p.m.

#### Example 2

65 At the stage after the addition of silver nitrate in the preparation of an high-speed photographic negative emulsion, 2 ml. per 100 ml. of the emulsion of a 1% aqueous solution of the compound (IV) was added. The emulsion was then added with stirring with a known precipitant (naphthalene-sulfonic acid-formalin resin), thereby to effect precipitation of light-sensitive silver halide crystals.

5

nize no substantial formation of foams. During the course of the emulsion preparation, samples were occasionally withdrawn and were subjected to foaming tests in the same manner as in the test B, thereby to obtain the results as shown below.

|                                      | Amount of foams<br>after silver salt<br>addition (ml.) |                 | Amount of foams<br>after first dispersion<br>of emulsion (ml.) |                 | Amount of foams<br>after finishing of<br>emulsion (ml.) |                 |
|--------------------------------------|--------------------------------------------------------|-----------------|----------------------------------------------------------------|-----------------|---------------------------------------------------------|-----------------|
|                                      | After<br>1.5 min.                                      | After<br>5 min. | After<br>1.5 min.                                              | After<br>5 min. | After<br>1.5 min.                                       | After<br>5 min. |
| Incorporated with compound (IV)----- | 0                                                      | 0               | 0                                                              | 0               | 16                                                      | 0               |
| Not incorporated-----                | 21                                                     | 7               | 26                                                             | 17              | 26                                                      | 14              |

The run in which the compound (IV) was used was entirely safe from foaming during the preparation of the photographic emulsion. The foaming after finishing of the emulsion was ascribable to the fact that a more or less amount of the compound (V) was lost due to water washing. 2

### Example 3

1.5 ml. of a 4% aqueous saponin solution and 4.5 ml. of a 1% aqueous solution of the compound (III) were added to 50 ml. of a high-speed negative photographic emulsion. As controls, another emulsion incorporated with only saponin and still another emulsion not incorporated with any of these were prepared. 25

These three emulsions were subjected to foaming tests in the same manner as in Example 2 to obtain the results as shown below.

| Agent used                      | Amount of foams (ml.) |              |
|---------------------------------|-----------------------|--------------|
|                                 | After 1.5 min.        | After 5 min. |
| Not incorporated-----           | 30                    | 24.5         |
| Saponin-----                    | 100                   | 62           |
| Saponin and compound (III)----- | 4                     | 4            |

These emulsions were coated, respectively, on a film base and then dried. The resulting light-sensitive photographic films were subjected to sensitometry to obtain the following results:

| Agent used                      | Photo-graphic speed | Fog  | Photo-graphic gamma |
|---------------------------------|---------------------|------|---------------------|
| Not incorporated-----           | 100                 | 0.10 | 0.66                |
| Saponin-----                    | 100                 | 0.10 | 0.65                |
| Saponin and compound (III)----- | 105                 | 0.11 | 0.68                |

Further, the appearance of these films was as follows:

| Type of emulsion                                      | Unevenness                                                                                              | Comet |
|-------------------------------------------------------|---------------------------------------------------------------------------------------------------------|-------|
| Not incorporated.....                                 | Coating was greatly coarse and was marked in unevenness or comet. Practically no com-<br>mercial value. | 5     |
| Incorporated with only saponin.....                   | Little.....                                                                                             | None. |
| Incorporated with saponin and com-<br>ound (III)..... | do.....                                                                                                 | Do.   |

As is clear from the above, the present invention inhibits the foaming of emulsions without giving any adverse effect to the photographic characteristics of the emulsions, and enables us to obtain photographic products with good quality.

6

### Example 4

3 ml. of a 4% aqueous solution of sodium isoamyl-dodecylsulfosuccinate (hereinafter referred to as "S") and 6 ml. of a 1% aqueous solution of the compound

(VII) were added to 100 ml. of a gelatino silver chloride photographic emulsion. A part of the mixture was used as a sample and was measured in formability in the same manner as in Example 2 to obtain the results as shown below. Further, the above emulsion incorporated with only S was used as a control.

|                                             | Volume of foams (ml.) |               |
|---------------------------------------------|-----------------------|---------------|
|                                             | After 5 min.          | After 10 min. |
| Incorporated with S and compound (VII)----- | 42.0                  | 35.5          |
| Incorporated with only "S"-----             | 72.6                  | 68.5          |

Subsequently, the emulsion incorporated with S and the compound (VII) was applied onto a baryta paper, and the resulting emulsion layer was further coated with a protective emulsion containing 1 ml. of a 1% aqueous solution of the compound (VII) and 0.5 ml. of a 4% aqueous solution of S. No repellency and unevenness were observed in wet-on-wet double coating. However, when a protective layer incorporated with only S is applied onto an emulsion layer incorporated with only S, repellency and unevenness was observed.

What we claim is:

1. A photographic gelatinous coating composition, which contains as an anti-foaming agent, a compound of the general formula



wherein  $n$  is an integer of 3 or 4 and  $m$  is an integer of not less than 5.

2. A photographic gelatinous coating composition as claimed in claim 1, wherein said composition is light-sensitive gelatino silver halide photographic emulsion.

## References Cited

UNITED STATES PATENTS

- 2,240,472 4/1941 Swan ----- 96-94  
2,768,894 10/1956 Harriman ----- 96-94

60 J. TRAVIS BROWN, Primary Examiner

U.S. Cl. X.R.

106—125